

## UNITED STATES PATENT OFFICE

2,265,202

CREPE THREAD AND METHOD OF MAKING  
SAME

George Schneider, Montclair, N. J., and William Whitehead, Rye, N. Y., assignors to Celanese Corporation of America, a corporation of Delaware

No Drawing. Application February 21, 1939,  
Serial No. 257,660

11 Claims. (Cl. 57—140)

This invention relates to the manufacture of crepe threads of organic derivatives of cellulose and to the production therefrom of fabrics exhibiting crepe effects.

An object of this invention is the economic and expeditious production of crepe yarns or threads containing organic derivatives of cellulose and which are suitable for the production of crepe fabrics.

A further object of this invention is the production of crepe yarns or threads which shrink and buckle with a lower degree of twist, or in shorter periods of time, or at lower temperatures when treated in a creping bath.

Other objects of this invention will appear from the following detailed description and the appended claims.

It has been previously found that if yarns of cellulose acetate or other organic derivative of cellulose have a high twist imparted thereto in the presence of hot aqueous media, such as steam or hot water, they produce crepe effects in fabrics containing them when given treatment in hot scouring baths.

We have found that if filaments, yarns or threads of organic derivative of cellulose have incorporated therein a crepe promoting agent, comprising a substance having a delayed solubility in water, prior to their being twisted in the presence of hot aqueous media, such as steam or hot water, many advantageous results are obtained. Thus, cellulose acetate yarn treated with our crepe promoting agent and then twisted in the presence of hot aqueous media produces at least as good crepe effects as cellulose acetate yarn that has not been treated with our agent prior to the twisting in presence of the aqueous media when (1) it contains less twist, say 10-15 turns per inch less, (2) fabric containing it is treated in a creping bath of 15 to 20° C. lower (80° to 85° C. as against boiling temperature), whereby delustering of the fabric may be avoided, (3) the time of treatment in the boil-off bath is reduced considerably, say to 10 to 20%.

In carrying this invention into effect, filaments, yarns or threads of any organic derivative of cellulose may be employed in the manufacture of the new crepe threads, for example, filaments, yarns or threads containing cellulose esters such as cellulose acetate, cellulose butyrate and cellulose propionate, and cellulose ethers such as ethyl cellulose and benzyl cellulose. The invention, however, is of especial value and will be described more particularly in connection with the

production of crepe yarns or threads of cellulose acetate.

As stated above, the crepe promoting agent that is incorporated with or applied to the filaments or yarns in accordance with this invention comprises a substance that has delayed solubility in water, by which is meant a substance of colloidal nature which is not freely soluble in water, but which when treated with water, especially at the temperature of the creping bath, absorbs water and swells. Examples of the crepe promoting agents that may be employed in this invention are proteins, whether of animal or vegetable origin such as proteins obtained from soya beans, gelatin or modified gelatin, or other albumens such as egg albumen, casein, and sericin; proteins which have been treated with formaldehyde or other aldehydes; gums, such as gum tragacanth; starches; methyl cellulose that swells in hot water; alkali soluble cellulose ethers such as ethyl cellulose and hydroxy ethyl cellulose.

In carrying out this invention any appropriate means may be employed for applying the crepe promoting agent to the filaments, yarns or threads. For example, the crepe promoting agent may be added to the spinning solution or dope from which the filaments constituting the yarns or threads are formed. We prefer, however, to apply the crepe promoting agent to the filaments, yarns or threads while they are travelling by passing them in contact with rollers, rods, pads or other devices supplied or impregnated with the crepe promoting agent, or by dipping the materials in the form of hanks in a bath containing the crepe promoting agent. In our preferred form of applying the agent to the materials, it is applied thereto in the form of an emulsion in water with or without an emulsifying agent such as a sulphated higher fatty alcohol or a salt thereof.

The emulsion employed in accordance with this invention contains such concentration of the crepe promoting agent as to impart thereto a consistency that is convenient. The amount of this emulsion to be applied to the filaments, yarns or threads of cellulose acetate is such that from 1 to 10% of the crepe promoting agent, based on the weight of the cellulose acetate, is retained thereon, depending upon the nature of the agent employed.

As stated above, the filaments, yarns or threads coated or impregnated with the crepe promoting agent are twisted in the presence of hot aqueous fluids such as steam or hot water, for instance, as is described in U. S. Patents Nos. 2,088,628 and

2,089,191. This twisting may be effected on a device of the kind in which the thread is drawn off over the head of a rotating package through a guide fixed substantially in line with the axis of rotation of the package and is thereafter wound on a bobbin or the like, the thread being passed through hot aqueous fluid on its way from the guide to the bobbin. In this way the yarn is subjected to the action of the hot aqueous fluid during the actual application of twist. The twisting spindle, the guide fixed in line with the axis of the spindle and the device for applying the hot aqueous fluid to the filaments, yarns or threads should be so arranged that the twist resulting from the rotation of the package is at least partially inserted while the thread is in contact with the hot aqueous fluid.

Where steam is employed as the hot aqueous fluid, steaming may conveniently be effected by allowing the thread to pass through a suitable chamber supplied with steam, preferably under such conditions that moisture is present. The chamber is provided with small holes, top and bottom, to permit passage of the thread, and also with a steam inlet. If desired, a single steam chamber may be arranged to serve a number of twisting devices, being provided with inlet and outlet holes for the thread of each twisting device. Such an apparatus may conveniently consist of a horizontal pipe mounted over a row of twisting devices and provided with eyes of porcelain, stainless steel, or other suitable material at appropriate points on top and bottom for the entrance and exit of the threads. The diameter of the pipe should be such as to afford the thread the requisite length of travel in the steam. Alternatively, a pipe having a smaller diameter may be used, in which case the pipe may be provided with hollow nipples communicating therewith and through which the yarn passes, the nipples being of sufficient length to provide, together with the diameter of the pipe, the requisite length of travel in the steam.

The presence of the desired moisture may be assured by supplying wet steam to the steaming device and/or by arranging for the condensation of steam to supply the requisite amount of moisture. For instance, small traps for condensed water may be provided at suitable intervals in the steaming chamber and steam injected therethrough by means of small pipes or orifices. Another method of insuring the presence of moisture is to wet the thread with water. For example, the bobbins of thread may be wetted before the twisting operation or, better, water may be applied to the thread by means of a wick or other device after the thread leaves the spindle and prior to its entering the steaming device.

Steam at slightly above atmospheric pressure, or at a pressure of 1 to 2 centimeters of water, is most conveniently employed. If desired, however, the steaming may be effected with steam at any desired super-atmospheric pressures, e. g. steam at 10 to 25 lbs. per square inch.

A steam treatment of relatively short duration, such as may be secured by causing the yarn to pass through steam in a path of about 1 to 6 inches at a speed of from 2 to 10 meters per minute has been found to give satisfactory results. Longer treatments may, however, be employed. For example, the yarn may be passed at the said speeds through 6 inches to 12 inches or more of steam.

The treatment of the thread with hot water during twisting may be effected by drawing the

thread off from a twisting spindle and passing it upwardly through a small hole in a suitable receptacle containing hot water, the thread then passing to a winding device. The hole may be, for example, about  $\frac{1}{2}$  of an inch in diameter and may be provided with means adapted to lead away and prevent from reaching the twisting spindle any liquid issuing from the hole. If desired, the hole may take the form of a short tube of fine bore, fixed in the receptacle, whereby the flow of liquid from the receptacle at the point of entrance of the thread may be reduced.

The duration of the treatment with hot water may be relatively short, such as may be secured when the thread is travelling at a speed of 2 to 10 meters per minute and is in contact with hot water for 1 to 3 inches of its travel. More prolonged treatments may, however, be employed.

Very good results may be obtained by using hot water at temperatures of 85 to 100° C. Preferably the water should be as hot as possible and temperatures of, for instance, 95 to 100° C. are to be recommended. If desired, the hot water may be employed under pressure, for example 2 to 10 or 15 pounds or more per square inch. The use of pressure enables the water to be employed at higher temperatures than is possible under atmospheric pressure. By using pressure, therefore, the temperature of the water may be above 100° C. and to the boiling point thereof at the pressure employed. Water may be employed under pressure, however, when the temperature is below 100° C.

The crepe twisting may be applied in a single stage. If desired, however, the crepe twist may be applied in two or more stages, at least the final stage of twisting being effected while treating the thread with hot aqueous fluid, as described in U. S. Patent No. 2,088,587.

When the crepe twist is applied in two or more stages the advantages of the process may be obtained when not only the final stage of the crepe twisting but the earlier stage or stages of twisting are also effected while treating the thread with hot aqueous fluid. In fact, it is of great advantage to effect, while treating the thread with hot aqueous fluid, any application of twist beyond the point at which twisting would result in weakening of the thread if the said twisting were effected without the hot aqueous fluid treatment.

The total twist applied in accordance with the process of the present invention may vary within wide limits, and the crepe figure in the fabric may be regulated according to requirements. The total twist desirable in any particular case depends upon a number of factors, including the precise effects required, the number of filaments, and the denier of the thread.

An important advantage of our process is that good crepe effects may be obtained with cellulose acetate yarn of lower degree of twist than has been attainable heretofore. Thus cellulose acetate yarn made in accordance with our invention having as low as 55 turns per inch can produce good crepe effects. The number of turns to be employed may be from 55 to 90 turns per inch, depending on the effects desired, the greater the number of turns, the less temperature and/or time of treatment being required in the creping bath.

While the process of this invention enables production of threads which yield satisfactory crepe effects without a special treatment, other than the twisting and hot aqueous fluid treatment characteristic of the process, other treat-

ments may, if desired, be employed further to improve the properties of the crepe threads and/or fabrics produced therefrom. Thus enhanced crepe effects may be obtained by treating the fabrics containing the crepe threads with aqueous solutions of saponifying agents such as the hydroxide or carbonates of sodium potassium or ammonium to superficially saponify the cellulose acetate yarns, prior to treatment with the creping bath. A convenient and effective method of doing this is to pad the fabric with an aqueous solution of an alkaline material, say a solution containing 15 to 40 grams per liter of sodium hydroxide and then drying the fabrics on heated cans.

The highly twisted crepe threads may be incorporated in the fabrics in various ways, for example, the weft alone may be wholly or partially composed of such threads or the warp may also contain them. Valuable fabrics may be produced by employing warp threads of relatively low twist and in the weft both crepe threads having a left-hand twist and crepe threads having a right-hand twist, pairs of threads of left-hand twist alternating with pairs of threads of right-hand twist.

If desired, the cellulose acetate crepe threads may be associated in the fabrics with highly twisted crepe threads of other materials, e. g. of natural silk or regenerated cellulose, or with highly twisted threads produced by other processes. Where the fabrics contain threads of low twist these may be wholly of cellulose acetate or wholly or in part of other materials, e. g. natural silk or regenerated cellulose.

Fabrics containing highly twisted crepe threads prepared in accordance with the invention may be subjected to a hot aqueous treatment in the manner commonly adopted in connection with fabrics comprising highly twisted yarns of natural silk. A particular advantage of this invention is that creping baths of relatively low temperature, say 80 to 85° C., may be used whereby the delustering of the cellulose acetate yarn may be avoided. However, if it is desired to decrease the time of treatment, creping baths of higher temperature up to the boiling point may be used, in which case the delustering effect of the hot aqueous baths upon fabrics containing lustrous threads of cellulose acetate may be minimized by the addition of salts or sugars to the baths.

In order to illustrate our invention, but not by way of limitation, the following examples are given:

*Example I*

Three pounds and five ounces of gelatin are stirred with twenty-nine pounds and eleven ounces of cold water. After standing at room temperature for 24 hours, the mixture is heated for one hour to 65-75° C. to complete the solution of the gelatin. The solution is cooled to 40° C. and thereupon there are added 12.5 cc. of glycerine, 46 cc. of 40% formaldehyde and 231 cc. of a 10% aqueous solution of Brilliant Avirol L-144WD (a sodium salt of sulfated higher fatty alcohol). This solution contains approximately 10% of solids.

Yarn of 166 denier comprising 40 filaments of acetone soluble cellulose acetate is dipped in the form of hanks in the above solution at 45 to 50° C., the hanks are then centrifuged down to about one and one-half times their original weight and dried in the air. This applies 5% of solids to the yarn. The hanks are then backwound onto bob-

bins. From these bobbins the yarn is twisted in the presence of steam to 70 turns per inch.

The so treated and twisted yarn is then woven as weft of 64 picks per inch into a fabric with a warp comprising 108 ends per inch of ordinary cellulose acetate, of 100 denier having 3 to 5 turns per inch, weft yarn of right-hand twist alternating with weft yarn of left-hand twist. The fabric is woven to a width of 45 inches. When this fabric is treated in a hot scouring creping bath good crepe effects are obtained. Thus a treatment for 15 minutes in a creping bath of 80-85° C. causes the original 45 inch wide fabric to shrink to a width of 33 to 34.5 inches, a treatment for 15 minutes in a creping bath of 98-100° C. causes shrinkage to 29-30 inches in width, while treatment for 2 hours in creping bath of 98-100° C. causes shrinkage to 28-29 inches in width.

*Example II*

The process of Example I is carried out, but before the fabric is subjected to the creping bath, it is padded with a saponifying agent comprising an aqueous solution containing 25 grams of sodium hydroxide per liter and then dried on cans. When this fabric is treated for 2 hours in a creping bath of 98° to 100° C., the fabric of an original width of 45 inches shrinks to a width of 27 inches.

*Example III*

The cellulose acetate yarn of Example I is treated with an aqueous solution of the isolated protein derived from soya bean, the amount applied being 5% of the weight of the fabric. This is crepe twisted in the presence of steam to 70 turns per inch and then woven into a fabric as described in Example I. When the fabric of 45 inch width is subjected to a creping bath of 98 to 100° C., it shrinks to a width of 17.5 inches when the treatment is for 15 minutes, and to a width of 14 inches when the treatment is for 2 hours.

It is to be understood that the foregoing detailed description is given merely by way of illustration and that many variations may be made therein without departing from the spirit of our invention.

Having described our invention, what we desire to secure by Letters Patent is:

1. Process for the production of crepe yarn of filaments of an organic derivative of cellulose, which comprises incorporating in the yarn a crepe promoting agent comprising a substance having a delayed solubility in water and crepe twisting the yarn while it is subjected to the action of a hot aqueous fluid.

2. Process for the production of crepe yarn of filaments of cellulose acetate, which comprises incorporating in the yarn a crepe promoting agent comprising a substance having a delayed solubility in water and crepe twisting the yarn while it is subjected to the action of a hot aqueous fluid.

3. Process for the production of crepe yarn of filaments of an organic derivative of cellulose, which comprises incorporating in the yarn a crepe promoting agent comprising a protein and crepe twisting the yarn while it is subjected to the action of a hot aqueous fluid.

4. Process for the production of crepe yarn of filaments of cellulose acetate, which comprises incorporating in the yarn a crepe promoting agent comprising a protein and crepe twisting the yarn while it is subjected to the action of a hot aqueous fluid.

5. Process for the production of crepe yarn of filaments of an organic derivative of cellulose, which comprises incorporating in the yarn a formaldehyde treated protein and crepe twisting the yarn while it is subjected to the action of a hot aqueous fluid.
6. Process for the production of crepe yarn of filaments of cellulose acetate, which comprises incorporating in the yarn a formaldehyde treated protein and crepe twisting the yarn while it is subjected to the action of a hot aqueous fluid.
7. Process for the production of crepe yarn of filaments of cellulose acetate, which comprises incorporating gelatin in the yarn and crepe twisting the yarn while it is subjected to the action of a hot aqueous fluid.
8. Process for the production of crepe yarn of filaments of cellulose acetate, which comprises incorporating formaldehyde treated gelatin in the
- 5      yarn and crepe twisting the yarn while it is subjected to the action of a hot aqueous fluid.
9. Process for the production of crepe yarn of filaments of an organic derivative of cellulose, which comprises incorporating in the yarn a protein derived from soya beans and crepe twisting the yarn while it is subjected to the action of a hot aqueous fluid.
10. Process for the production of crepe yarn of filaments of cellulose acetate, which comprises incorporating in the yarn a protein derived from soya beans and crepe twisting the yarn while it is subjected to the action of a hot aqueous fluid.
11. Crepe yarns of filaments of cellulose acetate and having a protein derived from soya beans incorporated therein.

GEORGE SCHNEIDER.  
WILLIAM WHITEHEAD.